

Feb. 4, 1941.

A. W. UELLENDAHL

2,230,788

STIFFENING MEMBER

Filed Aug. 25, 1939

Fig. 1.



Fig. 2.



Fig. 4.



Fig. 3.



Fig. 5.



Fig. 6.



Fig. 7.

WITNESSES

Geo. W. Maylor

J. H. Kane

INVENTOR

Arthur W. Uellendahl

BY

Munn, Anderson & Ladd

ATTORNEYS

## UNITED STATES PATENT OFFICE

2,230,788

## STIFFENING MEMBER

Arthur W. Uellendahl, Kew Gardens, N. Y., assignor to Barthels Manufacturing Company, Inc., Glendale, Brooklyn, N. Y., a corporation of New York

Application August 25, 1939, Serial No. 291,865

4 Claims. (Cl. 2-258)

This invention relates to an improved stiffening member, particularly to stiffening members of the type which may be used in association with garments, belts, cuffs, collars, or the like.

5 It is an object of the invention to provide an improved stiffening member having the desired character of stiffness so that it will serve in the proper manner to stiffen and reenforce the garments or other articles with which it is used but which nevertheless is flexible so that it may bend or yield in response to excess pressure without breaking and is resilient so that it will return to its normal position when the pressure is released.

10 Another object is the provision of an improved method or process of manufacturing a stiffening member of the above character.

In the accompanying drawing—

Fig. 1 is a plan view partially broken away of a 20 stiffening member embodying the present invention;

Fig. 2 is a side view partially broken away of the stiffening member;

Fig. 3 is a sectional view on the line 3—3 of Fig. 1;

Fig. 4 is a perspective view showing a portion of the stiffening rib in an intermediate stage in the manufacture thereof;

Fig. 5 is a fragmentary perspective view of an 30 outer casing which may be used in connection with my improved stiffening rib;

Fig. 6 is a fragmentary perspective view of a portion of a sheath used in connection with my stiffening rib; and

Fig. 7 is a fragmentary perspective view of one 35 of the types of stiffening strip which may be used in connection with this device.

My improved stiffening member preferably embodies one or more relatively thin, stiff, but nevertheless flexible and resilient strips which are encased in a sheath of textile fabric formed of threads of a plastic material which are partially disintegrated so as to cause the sheath to shrink and tightly engage the strip and to weld or bind the entire assembly into a unitary mass. An outer casing in the form of a fabric tube may then be placed around the assembly.

As the stiffening strips I use one or more strips 40 made of a resisting stiff material but which is nevertheless flexible so that it will yield without breaking when excess pressure is applied to it and which is also resilient or springy so that it will return to its normal position when the pressure is released. For this purpose I may employ 45 strips formed of cellulose or cellulose compounds

such as pyroxylin, cellulose acetate or the like. However, I prefer to employ a laminated strip of the type disclosed composed of two thin surface layers 11 made of regenerated cellulose such as "Cellophane" and an intermediate layer 12 5 made of ramie or similar fiber adhesively secured together in a well-known manner. Laminated "Cellophane" of this character is well known to those skilled in the art and is commercially available.

10 As previously stated I may employ one or more strips although as a practical matter I have found that for most purposes it is desirable to employ a plurality of strips in order to obtain the desired stiffness. For example, in the accompanying drawing I illustrate four strips which in practical experience has produced satisfactory results.

The stiffening strips 10 are arranged in superimposed fashion and are inserted in a sheath 14 20 formed of a fabric tube of a sufficient diameter to receive the strips and leave a slight clearance as shown in Fig. 4. The fabric tube may be made in any desired fashion but is preferably made on a braiding machine and it is formed of 25 threads of plastic material such as cellulose esters and for this purpose I prefer to employ cellulose acetate. Where the tube is made on a braiding machine the superimposed strips 10 may be used as a core and the tube may be 30 braided directly around the strips. After the strips 10 have thus been encased in the sheath 14 they are secured together and to the sheath by means of a line of stitching 15 as shown most clearly in Fig. 4.

35 Thereafter the material forming the threads of sheath 14 is partially plasticized and then dried with the result that the sheath shrinks and tightly engages the encased strips and the entire assembly is welded into a unitary structure by means of the plastic material. The plasticizing action may result either from a suitable solvent for the plastic material or from heat where a thermo-plastic material is employed.

40 As stated above, in the preferred form of my invention the threads are made of cellulose acetate and in this instance to plasticize the material the assembly of strips and sheath are preferably passed through a bath containing a suitable cellulose acetate solvent such as a mixture 45 of acetone and alcohol, a mixture of alcohol and chloroform, or alcohol and benzol, or glacial acetic acid. After passing through the bath the cellulose acetate yarns are partially plasticized 50 so that some of the plastic material enters the 55

interstices in the sheath and between the strips and the sheath. Thereafter the solvent is evaporated away as by the application of heat which may be accomplished by passing the assembly through heated ducts. When the solvent has evaporated away, the sheath 14 shrinks to a size to tightly engage the stiffening strips 10 and the cellulose acetate which was plasticized serves as a filler and binding agent as indicated by the small dots in Figs. 1, 2 and 3, stiffening and reenforcing the sheath and binding the entire assembly into a unitary structure.

After the assembly has been thus treated it may be used directly without any further treatment as a stiffening member or, if preferred, it may be encased in a fabric tube 16 which may be composed of two strips of textile fabric such as woven cotton secured together along their longitudinal edges at the two sides of the stiffening strip, as indicated at 17.

My improved stiffening strip may be used in a well-known manner in connection with foundation and other undergarments or in connection with outer garments. It may also be used to stiffen and reenforce belting, cuffs, collars, and in other associations where stiffening members are employed.

It will be appreciated from the foregoing description of my invention that I have provided an improved stiffening agent having the desired characteristics of stiffness and resiliency and which is relatively inexpensive and may be manufactured from materials which are readily available. It will also be appreciated that I have provided an improved process for manufacturing stiffening members of the above character which is relatively simple to carry out and requires a minimum of labor.

While I have illustrated and described a preferred embodiment of my invention it should be understood of course that modifications may be made without departing from the invention as set forth in the accompanying claims.

I claim:

1. A stiffening member comprising a plurality of superimposed thin, elongated strips formed of a stiff resilient cellulose material, a fabric sheath formed of threads of plastic material tightly encasing the strips, and stitching securing the strips and sheath together, the threads of the sheath being partially disintegrated so that the plastic material thereof serves as a filler to stiffen and reenforce the sheath and as a binder to bind the strips and sheath into a unitary structure. 5

2. A stiffening member as set forth in claim 1 in which the strips are made of laminated plies of regenerated cellulose and fiber and the threads of the fabric sheath are made of cellulose acetate. 15

3. The method of making a stiffening member which comprises first providing a plurality of relatively thin, elongated strips of stiff resilient cellulose material and a sheath formed of threads of plastic material, then encasing the strips in 20 the sheath and securing them together by means of stitching, next, partially plasticizing the threads of the sheath so as to cause the sheath to shrink and so as to cause the plastic material to flow into the interstices in the sheath and between the strips and sheath, and finally solidifying the plastic material so as to cause the plasticized portion thereof to serve as a filler to stiffen and reenforce the sheath and as a binder to bind the strips and sheath into a unitary structure. 25 30

4. An elongated stiffening member comprising a plurality of superimposed thin elongated laminated strips each formed of layers of regenerated cellulose and fiber, a fabric sheath formed of threads of plastic material tightly encasing the strips and stitching securing the strips and sheath together, the threads of the sheath being partially disintegrated so that the plastic material thereof serves as a filler to stiffen and re-enforce the sheath and as a binder to bind the strips and sheath into a unitary structure. 40 35

ARTHUR W. UELLENDALH.